

March 31, 1925.

1,531,472

E. E. BAKER

METHOD AND APPARATUS FOR SHAPING METALS

Filed Oct. 10, 1921



Inventor  
Ernest E. Baker  
By Miller Chindahl Parker  
Attest

Patented Mar. 31, 1925.

1,531,472

# UNITED STATES PATENT OFFICE.

ERNEST E. BAKER, OF CHICAGO, ILLINOIS.

## METHOD AND APPARATUS FOR SHAPING METALS.

Application filed October 10, 1921. Serial No. 506,565.

*To all whom it may concern:*

Be it known that I, ERNEST E. BAKER, a citizen of the United States, residing at Chicago, in the county of Cook and State 5 of Illinois, have invented an Improved Method and Apparatus for Shaping Metals, of which the following is a specification.

The invention relates to an improved method and apparatus for shaping molten 10 metal whereby a continuous operation in the nature of die-casting may be accomplished to advantage.

The die-casting operation as heretofore carried out, has, so far as I am aware, been 15 limited to the introduction of the metal to be formed into a stationary die or mold, in which the metal is confined until cool. It is obvious, therefore, that the length of the article or product to be cast is necessarily 20 limited. Moreover, the cost of producing articles relatively large in size is often prohibitive. In accordance with my invention 25 the operation is rendered continuous by effecting relative movement between the metal as it becomes plastic and a die block or mold. Accordingly, an article of any desired or varying lengths may be produced by the same forming means.

The aim of the invention, therefore, 30 generally stated, is to provide a method and apparatus by which a continuous shaping or casting operation may be performed with a resulting increase in the quality of the completed product and in the efficiency of the operation, the cost as compared with the benefits obtained being relatively slight.

With this aim in view, the invention consists in the deposit of a steel alloy or other metal in molten form upon a base or support of suitable material, by introducing such metal into a die block or mold surrounding or enclosing a portion of the base, and effecting relative motion between the mold and the base whereby the desired 45 form or shape is imparted to the deposited metal as it becomes cooled and hence plastic in its passage through the mold.

A specific application of the invention 50 consists in the deposit of a desired metal upon a base in the form of a member or part previously formed, in order to form an integral part thereof. This is accomplished by effecting the adhesion of the molten metal upon its introduction into 55 the mold or die to such part, as by raising

the surface temperature thereof to the fusion point as it becomes enclosed by the mold. For example, a steel alloy, such as manganese steel, may be applied to a previously formed or rolled steel railroad rail, 60 thus providing a head of high wear-resisting qualities.

In the accompanying drawings I have illustrated one embodiment only of my invention, in connection with a rolled steel 65 rail, forming the base or support, to which is applied a wear-resisting surface composed of a steel alloy such as manganese steel. I desire to point out, however, that while the invention is thus illustrated and herein described, it is susceptible of wide and varied usage, and various changes in the form, construction, arrangement of the parts and mode of operation may be made without departing from the spirit and scope of the 75 invention as expressed in the appended claims.

In Figure 1 of the drawings I have shown in side elevation a view somewhat diagrammatic in character illustrating an apparatus 80 whereby my invention may be carried out. Fig. 2 is a transverse vertical sectional view taken in the plane of line 2-2 of Fig. 1. Fig. 3 is a fragmentary longitudinal vertical sectional view taken approximately in 85 the plane of line 3-3 of Fig. 2. Fig. 4 is a fragmentary plan view of a portion of the apparatus.

Referring first to Figure 1, A designates a railroad rail which is mounted for movement with respect to a shaping or forming device 7, and 8 indicates a crucible for molten metal. 9 and 10 designate, respectively, heating stations for the heat treatment of the rail prior to its passage into 95 the device 7, and prior to its passage beneath a cooling means 11.

Any suitable means may be employed for effecting the movement of the rail A at a predetermined rate of speed through the device 7. Herein I have shown, by way of example, a plurality of rolls 12, mounted upon horizontal axes and upon which the rail is adapted to rest. Feeding and guiding means are provided for engaging the side of the rail. This means may comprise a plurality of rollers 13 mounted on vertical shafts 17 the lower ends of which are geared to the horizontal drive shaft 18.

The device 7 (Figs. 2 and 3) consists of a die

- block or mold such, for example, as the member 19, made from carbon or other heat-resisting material and constructed to provide an interior surface in the form of a through passageway 20 therein. The forward end 20<sup>a</sup> of this passage is made of a size adapted to receive snugly the body of the rail A, and opening into the forward portion of the passageway is a pouring slot 21. To prevent the rail from sticking in the mold because of the snug fit provided between it and the rail at the end 20<sup>a</sup> of the passageway 20, graphite or other suitable lubricant may be supplied at this point under high pressure.
- 10 As shown in said figures, the portion of the passageway rearwardly of the restricted forward end is shaped so that when the rail head is in position within the die-block a space is provided between the upper surface of the rail and the upper walls 20<sup>b</sup> of the passageway, and said walls are so shaped as to form the metal introduced into the mold into a layer or strip B of the desired exterior conformation.
- 15 Herein, the die block is supported in position by means of a suitable clamp or frame 22, having bolts 23 for engaging the sides of the block.
- 20 The crucible 8 may be of any suitable character adapted to supply a continuous stream of molten metal to the die-block. Also, any suitable means may be provided for supporting the crucible in the proper relation to the die-block.
- 25 In order to effect the adhesion of the metal poured into the die-block to the rail, or other member passing therethrough, I provide suitable heating means 9. This means, as herein shown, consists of a pair of gas burners 24, although it will be understood that any form of heating means may be employed which is capable of raising the surface temperature of the member being treated to the fusion point.
- 30 It will be understood that the speed at which the rail A passes through the die-block 19 is determined in accordance with the time required to heat the surface thereof to the fusion point, and the rapidity with
- 35 which the molten metal becomes plastic so as to be capable of being properly shaped, it being obvious that when the molten metal is introduced through the pouring slot, it immediately unites with the metal of the rail and thus adheres thereto, becoming an integral part of it. As herein shown, the rail A is made from rolled steel in the usual way, except that its head is made of less thickness, with a flattened top surface to
- 40 which is applied the layer or strip B of steel alloy.

Preferably, the burners are of such a character as to apply an intense heat capable of quickly penetrating to the desired depth in the time consumed in its passage therebe-

neath. Thus the surface only of the rail is affected by the heat from the burners 24, and there is therefore no tendency of the rail to become distorted or otherwise injured.

70 It will be observed that the interior of the die block rearwardly of the pouring slot 21 is made of substantial length. Thus, as the rail passes through this portion of its travel through the die-block, the latter has 75 a cooling or chilling effect on the applied metal such that it becomes hardened. Thus, the die-block or mold constitutes a combined shaping and cooling device. Should such chilling of the metal be insufficient, additional means may be provided for this purpose, such, for example, as the heating means 10 and the cooling means 11. The means 10 may be in the form of burners 24<sup>a</sup>, and the cooling means may be of any suitable character such as a pipe 25 connected with a source of water supply and having jet openings arranged to discharge the cooling water onto the rail after it emerges 80 from beneath the burners 24<sup>a</sup>.

85 It will be apparent that a railroad rail or other member thus provided with a hardened or wear resisting surface is much superior to the ordinary steel rail, while the cost, owing to the simplicity of the treatment, is relatively small. Indeed, from the standpoint of quality alone, such an article is superior to one constructed wholly from the steel alloy, since only that portion of 90 the member which receives the wear is hardened, leaving the remaining portion in a relatively softer condition, and hence capable of being readily bent, drilled and the like. Thus, in the case of the railroad rail, the application of the wear-resisting metal does 95 not interfere in any way with the drilling of holes in the base of the rail for the reception of the connecting bolts, nor does it prevent the same from being cut or bent as 100 desired.

105 When the alloy is applied to the base so as to become a part thereof, as in the case of the railroad rail, it will be obvious that the rails are passed successively, end to end, through the die or mold, so as to render the 110 operation continuous. Accordingly, the applied metal emerges from the mold or die in a continuous strip, and must be severed before the rails can be separated. To ensure that the deposited metal will not cause the adhesion of the rails themselves at their adjacent ends, a suitable filler such as fire-clay 115 (not shown) may be interposed therebetween.

120 It will be understood that the invention herein illustrated and described in detail is not limited to the use of a specially formed rail such as the rail provided with a flattened head, for obviously by properly proportioning the parts, the alloy may be ap- 125

plied to articles which have become worn in usage, thus effecting a substantial renewal thereof.

- I desire to point out especially that while 5 I have herein shown a stationary shaping device, and a movable base or support, the invention is not limited to this particular arrangement, for obviously the reverse arrangement may be employed if desired. 10 Moreover, the apparatus herein shown is purely of an illustrative character, and its details form no essential part of the present invention.

I claim as my invention:

- 15 1. The method of applying an alloy such as manganese steel to a railroad rail or other article which consists in initially heating to a fusion point the surface which is to receive the alloy, depositing molten metal onto such 20 heated surface, confining the metal deposited on the heated surface, and then as the metal becomes plastic forming or shaping it while simultaneously cooling it to provide the desired contour to the completed article.
- 25 2. The method of making railway rails which consists in heating to the fusion point the substantially flat upper surface of a rail body formed from rolled steel, then deposit-

ing an alloy such as manganese steel in molten form onto such surface, and then causing 30 relative movement between the rail and a die so that as the metal becomes cool and plastic it is shaped by the die to produce a peripheral surface of the desired contour.

3. An apparatus of the character described comprising, in combination, a die block having a through passageway and a filling opening in one side thereof adapted for the insertion of molten metal, means for effecting relative longitudinal movement between said block and a part to be treated extending through said passageway, said passageway being shaped at one side of said opening to conform substantially to the shape of the part to be treated and at the 45 other side of said opening providing a forming and shaping wall of substantial length spaced from the part to be treated, and means for heating said part to the fusion point immediately prior to its entrance into 50 said passageway opposite said filling opening.

In testimony whereof, I have hereunto set my hand.

ERNEST E. BAKER.